

# United States Patent Office.

S. D. McPHERSON, OF NORMAL, ILLINOIS.

*Letters Patent No. 76,225, dated March 31, 1868.*

## IMPROVED COMPOUND FOR MAKING PICTURES TRANSPARENT.

The Schedule referred to in these Letters Patent and making part of the same.

### TO ALL WHOM IT MAY CONCERN:

Be it known that I, S. D. McPHERSON, of Normal, in the county of McLean, and in the State of Illinois, have invented certain new and useful Improvements in Compound for Making Pictures Transparent; and do hereby declare that the following is a full, clear, and exact description of the mode of compounding and using the same.

To prepare a small quantity of this compound, I use, first, balsam fir, two ounces; second, Demar varnish, one ounce; third, alcohol, half an ounce; fourth, turpentine, one ounce.

These ingredients, in the above proportions, are placed in a bottle, and well shaken. After they have become thoroughly united, which will be the case in a few moments, the compound is applied to the picture with an ordinary varnish-brush.

The picture is placed with its face downward and upon glass, or some equivalent substance. The compound is then put on the back of the picture, and renders it so transparent that the back can be readily painted in oil colors, thus giving the appearance of an oil-colored painting to the face.

What I claim, is—

The within-described ingredients, compounded and used substantially as and for the purpose set forth.

In testimony that I claim the foregoing, I have hereunto set my hand, this 19th day of October, 1867.

S. D. McPHERSON.

Witnesses:

JAMES W. BROWN,

A. N. MARR.